

March 13, 1956

W. VAN LOON ET AL

2,738,256

PREPARATION OF CALCIUM CARBIDE

Filed Dec. 28, 1953



Inventors  
Willem Van Loon  
Lieds Koopal  
By Cushman, Darby & Cushman  
Attorneys

1

2,738,256

## PREPARATION OF CALCIUM CARBIDE

Willem Van Loon, Geleen, and Sieds Koopal, Sittard, Netherlands, assignors to Stamicarbon N. V., Heerlen, Netherlands

Application December 28, 1953, Serial No. 400,769

Claims priority, application Netherlands  
December 30, 1952

2 Claims. (Cl. 23—208)

The invention relates to the preparation of calcium carbide in a shaft furnace by the process (hereinafter termed "the process as referred to") in which a mixture of a fuel mainly consisting of carbon, such as coke, charcoal or anthracite, and a calcareous compound to be converted into carbide such as unslaked lime, limestone or dolomite is fed into the shaft furnace at the top thereof, and the amount of heat and the temperature needed for the reaction between the carbon and the compound to be converted is produced by burning part of the fuel present by means of an oxygen-containing blast which is injected into the furnace through laterally positioned tuyeres. The product formed collects in the lower part of the shaft furnace in the so-called melt pot, from which it can be discharged through a tap hole, either continuously or periodically.

The invention relates in particular to the manner in which the oxygen-containing blast is fed into the shaft furnace.

Provision should be made for injecting the oxygen-containing blast so that, on leaving the tuyeres, the blast is distributed as uniformly as possible over the entire horizontal cross sectional area of the furnace in order to obtain a horizontal combustion zone of white-hot fuel.

In the case of blast furnaces this is effected by providing a ring of tuyeres which as a rule are placed in a horizontal position and through which the blast is supplied at a high rate (about 180 m./sec.). The draught in the furnace causes the blast to ascend as a result of which the combustion zone does not extend, or only extends but a short distance, downwardly from the tuyeres, and the fuel in front of the tuyeres is set in strongly turbulent motion.

It has now been found, quite unexpectedly, that in the preparation of calcium carbide, in a shaft furnace the process may be made to proceed more smoothly if the strongly turbulent motion of the fuel in front of the burners can be avoided or reduced. In particular the trouble that the charge of the furnace gets stuck or that even the entire furnace gets blocked if the fuel in the combustion zone is not set in strongly turbulent motion. The step of considerably lowering the injection velocity below the value which is customary as in the blast furnace production of iron, is not in itself sufficient however, since although this step avoids the turbulent motion referred to, the use of a low injection rate causes the formation of a peripheral fire instead of the desired horizontal combustion zone over the entire cross sectional area of the furnace.

### Objects

It is an object of the present invention to prepare calcium carbide in a shaft furnace by an improved method.

It is a further object to prepare calcium carbide in a shaft furnace in a way whereby the possibility of the charge getting stuck in the shaft furnace is avoided or strongly reduced.

It is another object of this invention to prepare calcium

2

carbide in a shaft furnace in which furnace the fuel in front of the tuyeres is not set in strongly turbulent motion.

A further object of this invention is in the preparation of  $\text{CaC}_2$  in a shaft furnace to inject the oxygen-containing blast so that on leaving the tuyeres the blast is distributed as uniformly as possible over the entire horizontal cross sectional area of the furnace.

Another object is to obtain in the furnace a horizontal elongated combustion zone of white-hot quietly moving fuel.

Still further objects and the entire scope of applicability of the present invention will become apparent from the detailed description given hereinafter.

### General description

These objects are accomplished according to the present invention by sloping the tuyeres downwardly towards their free ends.

This slope should not be so great, however, that the oxygen-containing blast comes into contact with the melt as this may lead to rapid oxidation of the molten product with deleterious effects upon the process as a result. It is found that a slope greater than  $30^\circ$  should be avoided.

Accordingly the present invention provides a process as referred to for the preparation of a carbide in a shaft furnace, in which the oxygen-containing blast is supplied at a velocity lower than 100 m./sec. and higher than 40 m./sec. through annularly arranged tuyeres the axes of which slope downwardly towards the free ends of the tuyeres at an angle of  $10^\circ$  to  $30^\circ$  to the horizontal.

It is preferred to keep the air blast velocity in the range of 50 to 80 m./sec. Velocities lower than 40 m./sec. are not suitable since in this case the oxygen does not penetrate far enough in a horizontal direction and a peripheral fire may form. If the angle between the tuyeres and the horizontal is greater than  $30^\circ$ , it is found that the permissible blast velocities are so low that a good result is not obtained. A reduction of the angle between the tuyere axes and the horizontal plane, below  $10^\circ$ , increases the danger of a peripheral fire unless the velocity of the blast is kept so high that a strong turbulence of the fuel in front of the tuyeres is set up which leads to segregation of the charge and the symptom of getting stuck of the charge.

The invention is illustrated by the accompanying drawing wherein a partial vertical section of the lower end of a shaft furnace is shown. The shaft furnace 1 is provided with a cooling spiral or coil 11 at the level of the combustion zone. Projecting into the furnace are a number of burners 12 through which the oxygen-containing blast is blown into the furnace via a ring conduit 15. The bottom of the shaft furnace is formed by the melting pot 20 from which the product formed is withdrawn through the tap hole 18.

According to the invention the angle between the axes of the burners and the horizontal amounts to  $10^\circ$ — $30^\circ$ .

### Conclusion

The present invention provides to a process for the manufacture of calcium carbide in a shaft furnace by starting from a mixture of solid fuel, mainly consisting of carbon, and a calcareous addition in which process part of the fuel present is converted to gases by an oxygen-containing blast in order to provide the amount of heat and the high temperature required for the formation of calcium carbide, which molten carbide is collected in the lower section of the furnace and which can be discharged either continuously or periodically; the process according to the invention being characterized by the fact that the oxygen-containing blast is supplied at a velocity lower than 100 m./sec. and higher than 40 m./sec. through annularly arranged tuyeres the axes of which

slope downwardly towards the free ends of the tuyeres at an angle of 10° to 30° to the horizontal. By operating in accordance with the present invention it is possible to prepare calcium carbide in a shaft furnace in a very smooth way without the trouble that the charge in the furnace gets stuck or that the furnace gets blocked.

We claim:

1. In a process for preparing calcium carbide in a shaft furnace from a mixture of a solid fuel comprising carbon, and a calcareous material and involving the steps of (a) 10 converting part of said fuel to gases with an oxygen-containing blast injected annularly into said furnace to provide the heat and temperature required for carbide formation, (b) permitting the resulting gas to escape through the top of the furnace while (c) collecting molten 15 carbide in the lower section of the furnace, the improve-

ments which comprise injecting the oxygen-containing blast into said furnace at a velocity of between 40 m./sec. and 100 m./sec. and at an angle of between 10° and 30° to the horizontal.

5 2. Process according to claim 1, wherein the injection velocity is higher than 50 and lower than 80 m./sec.

References Cited in the file of this patent

UNITED STATES PATENTS

|           |               |               |
|-----------|---------------|---------------|
| 826,743   | Price         | July 24, 1906 |
| 1,098,534 | Servais       | June 2, 1914  |
| 1,146,776 | Wallmann      | July 13, 1915 |
| 2,174,900 | Snyder        | Oct. 3, 1939  |
| 2,380,008 | Abrams et al. | July 10, 1945 |
| 2,476,760 | Ohlsson       | July 19, 1949 |